

## UNITED STATES PATENT OFFICE

2,613,205

PRODUCT OF REACTION OF PHOSPHORUS  
SULFIDE, AND HYDROCARBON, WITH  
GUANIDINE CARBONATE

Max W. Hill, Somerville, N. J., assignor to Standard Oil Development Company, a corporation of Delaware

No Drawing. Application April 23, 1949,  
Serial No. 89,370

16 Claims. (Cl. 260—132)

**1** This invention relates to mineral oil compositions and particularly to lubricants containing a detergent additive.

The art of metallic detergents for lubricating oil compositions adapted for use in internal combustion engines is well known to those versed in this field and has resulted in substantial improvements in lubricants. These detergents are particularly useful in lubricating oil compositions which are employed in internal combustion engines used in the operations of automobiles, aircraft and similar vehicles, including Diesel engines, to improve their operation by preventing or retarding corrosion, piston ring sticking, cylinder wear, and carbon and varnish formation. However, when metallic detergents are used in lubricating compositions where oil consumption is high and engine conditions are severe, such as in aircraft engines or where such concentrations of metallic detergents are used to maintain engine cleanliness under conditions where high deposit fuels of cracked or high sulfur nature are used, such as in automobile and Diesel operation, the ash content from the metallic detergent accumulates in the combustion chamber and causes pre-ignition, detonation, spark plug fouling, valve burning, and ultimate destruction of the engine.

It has been found, in accordance with the present invention, that if the reaction product of a phosphorus sulfide with an essentially hydrocarbon product is neutralized with guanidine or any of its derivatives as hereinafter defined or with any other compound containing a guanyl radical, the product so formed is very stable at the temperatures of engine operation and serves the purpose of a good detergent and anti-oxidant. When incorporated in mineral lubricating oil which is used in an internal combustion engine, and because it contains no metal, it is free from the objectionable feature of leaving a metallic deposit or ash. These compounds are effective not only when added directly to the crankcase lubricant but also when added to the engine fuel, since in the operation of the engine it will work its way from the combustion chamber into the crankcase and there blend with the lubricant.

Guanidine and guanidine derivatives may be employed as the basic reagents for neutralizing the titratable acidity of the phosphorus sulfide-hydrocarbon reaction product. The free base guanidine and its derivatives may be used as well as basic acting salts of such bases, by which is meant salts of acids whose strength, measured on a pH scale, is less than that of the acidic phosphorus sulfide-hydrocarbon product. Such

basic acting salts are, for example, the carbonates of guanidine and its derivatives. Alternatively, the final products may be formed by double decomposition of a salt of guanidine or guanidine derivative, e. g., guanidine hydrochloride or sulfate, with a metal salt of the phosphorus sulfide-hydrocarbon reaction product. Although guanidine and its salts are preferred, substituted guanidines may be used. Broadly, the guanidine type basic compounds which may be reacted in accordance with the present invention may be defined by the formula



in which R, R', and R'' represent hydrogen or hydrocarbon groups containing 1 to 20 carbon atoms, e. g., straight chain alkyl groups, such as methyl, ethyl, propyl, butyl, also higher straight and branched chain alkyl groups, such as octyl, isoctyl, 2-ethylhexyl, decyl, dodecyl, tetradecyl, cetyl and stearyl radicals. R, R' and R'' may also represent cycloalkyl, arylalkyl, aryl or alkylaryl groups, for example, methylcyclohexyl, phenylethyl, phenyl, cresyl, and tert.-butylphenyl groups. It will be understood that R, R' and R'' can be the same or different atoms or groups in the same molecule. However, in the case of a substituted guanidine it is most preferable to employ symmetrically tri-substituted compounds, and alkyl and cycloalkyl groups are the more preferred types of substituting groups. These include the symmetrical trialkyl, triarylpheyl, and triarylkyl guanidines. Also highly preferred classes of substituted guanidines include the monoalkyl, mononaphthyl, and mono-arylalkyl guanidines; unsymmetrical dialkyl, dinaphthyl, and diarylkyl guanidines. Somewhat less preferable but still useful classes are the symmetrical dialkyl, dinaphthyl, and diarylalkyl guanidines, and the mono-, di-, and triaryl guanidines. Still other substituted guanidines may be used, such as biguanide, dicyandiamide, and dicyandiamidine.

Specific examples of basic acting compounds illustrating the above-described types are the following:

- Guanidine
- α-Methylguanidine
- α-Ethylguanidine
- α-Hexylguanidine
- α-Heptylguanidine
- α-Phenyethylguanidine
- α-Benzylguanidine
- α-Cyclohexylguanidine

$\alpha$ -Decylguanidine  
 $\alpha$ -Hexadecylguanidine  
 $\alpha$ -Octadecylguanidine  
 $\alpha$ -Phenylguanidine  
 $\alpha, \alpha$ -Dimethylguanidine  
 $\alpha, \alpha$ -Diethylguanidine  
 $\alpha, \alpha$ -Diisooamylguanidine  
 $\alpha, \alpha$ -Dihexylguanidine  
 $\alpha, \alpha$ -Dihexylguanidine  
 $\alpha, \alpha$ -Diphenylethylguanidine  
 $\alpha, \alpha$ -Dibenzylguanidine  
 $\alpha, \alpha$ -Dicyclohexylguanidine  
 $\alpha, \alpha$ -Didecylguanidine  
 $\alpha, \alpha$ -Dihexadecylguanidine  
 $\alpha, \alpha$ -Dioctadecylguanidine  
 $\alpha, \alpha$ -Diphenylguanidine

The  $\alpha, \gamma$ -substituted guanidines corresponding to the above-listed  $\alpha, \alpha$ -substituted compounds.

The following symmetrical tri-substituted guanidines:

Trimethylguanidine  
 Triethylguanidine  
 Trioctadecylguanidine  
 Tricyclohexylguanidine  
 Tribenzylguanidine  
 Triphenylguanidine

Carbonates of any of the above-listed compounds.

The sulfide of phosphorus which is employed in the reaction with hydrocarbon material may be  $P_2S_3$ ,  $P_2S_5$ ,  $P_4S_3$ ,  $P_4S_7$  or other phosphorus sulfide, and is preferably phosphorus pentasulfide,  $P_2S_5$ .

The hydrocarbon material which may be reacted with a phosphorus sulfide in the first step of the production of additives of the present invention may be paraffins, olefins or olefin polymers, diolefins, acetylenes, aromatics or alkyl aromatics, cyclic aliphatics, petroleum fractions, such as lubricating oil fractions, petrolatums, waxes, cracked cycle stocks, or condensation products of petroleum fractions, solvent extracts of petroleum fractions, etc.

Essentially paraffinic hydrocarbons such as bright stock residuums, lubricating oil distillates, petrolatums or paraffin waxes may be employed. There may also be employed products obtained by condensing any of the foregoing hydrocarbons, usually through first halogenating the hydrocarbon, with aromatic hydrocarbons in the presence of anhydrous inorganic halides, such as aluminum chloride, zinc chloride, boron fluoride, and the like.

As examples of monoolefins may be mentioned isobutylene, acrolein, decene, dodecene, cetene ( $C_{16}$ ), octadecene ( $C_{18}$ ), cerotene ( $C_{26}$ ), melene ( $C_{30}$ ), olefinic extracts from gasoline or gasoline itself, cracked cycle stocks and polymers thereof, resin oils from crude oil, hydrocarbon coal resins, cracked waxes, dehydrohalogenated chlorinated waxes, and any mixed high molecular weight alkenes obtained by cracking petroleum oils. A preferred class of olefins are those having at least 20 carbon atoms per molecule, of which from about 12 to about 18 carbon atoms, and preferably at least 15 carbon atoms, are in a long chain. Such olefins may be obtained by the dehydrogenation of paraffin waxes, by the dehydrohalogenation of long chain alkyl halides, by the synthesis of hydrocarbons from  $CO$  and  $H_2$ , by the dehydration of alcohols, etc.

Another class of suitable olefinic materials are the monoolefin polymers, in which the molecular weight ranges from 100 to 50,000, preferably from about 250 to about 10,000. These polymers may

be obtained by the polymerization of low molecular weight monoolefinic hydrocarbons, such as ethylene, propylene, butylene, isobutylene, normal and isoamylenes, or hexenes, or by the copolymerization of any combination of the above monoolefinic materials.

Diolefins which may be employed include well known materials such as butadiene, isoprene, chloroprene, cyclopentadiene, 2,3-dimethylbutadiene, pentadiene-1,3, hexadiene-2,4, terpenes, and the like. Acetylene and substituted acetylenes may similarly be employed.

Another class of unsaturated hydrocarbon materials which may be advantageously employed in the preparation of the additives of this invention are high molecular weight copolymers of low molecular weight monoolefins and diolefins. The copolymer is prepared by controlled copolymerization of a low molecular weight olefin and a non-aromatic hydrocarbon showing the general formula  $C_nH_{2n-x}$ , in which  $x$  is 2 or a multiple of 2, in the presence of a catalyst of the Friedel-Crafts or peroxide type. The low molecular weight olefin is preferably an isolefin or a tertiary base olefin preferably one having less than 7 carbon atoms per molecule. Examples of such olefins are isobutylene, 2-methylbutene-1,2-ethylbutene-1, secondary and tertiary base amylene, hexamethylenes, and the like. Examples of the non-aromatic hydrocarbons of the above formula which can be used are the conjugated diolefins listed in the preceding paragraph, diolefins such as 1,4-hexadiene, in which the double bond is not conjugated, as well as the acetylenes. The copolymerization is preferably carried out in the presence of aluminum chloride, boron fluoride, or benzoyl peroxide, and the copolymer is preferably one having a molecular weight of about 1,000 to 30,000.

Another class of hydrocarbons which may be employed in a similar manner are aromatic hydrocarbons, such as benzene, naphthalene, anthracene, toluene, xylene, diphenyl, and the like, as well as aromatic hydrocarbons having alkyl substituents and aliphatic hydrocarbons having aryl substituents.

A still further class of hydrocarbons which may be employed in the reaction with sulfides of phosphorus are condensation products of halogenated aliphatic hydrocarbons with an aromatic compound, produced by condensation in the presence of aluminum chloride or other Friedel-Crafts type catalyst. The halogenated aliphatic hydrocarbon is preferably a halogenated long chain paraffin hydrocarbon having more than 8 carbon atoms, such as paraffin wax, petrolatum, ozocerite wax, etc. High viscosity paraffin oils, particularly heavy residual oil which has been treated with chemicals or extracted with propane or other solvents for the removal of asphalts, may be employed. The aromatic constituent may be naphthalene, fluoranthene, phenanthrene, anthracene, coal tar residues, and the like.

Another type of hydrocarbon material which may be similarly employed is a resin-like oil which has a molecular weight of from about 1,000 to 2,000 or higher, obtained preferably from a paraffinic oil which has been dewaxed and which is then treated with a liquefied normally gaseous hydrocarbon, e. g., propane, to precipitate a heavy propane-insoluble fraction. The latter is a substantially wax-free and asphalt-free product having a Saybolt viscosity at 210° F. of about 1,000 to about 4,000 seconds or more.

## 5

The additive employed in the present invention is the neutralized reaction product obtained by reacting one or more of the herein described hydrocarbons with a phosphorus sulfide, preferably phosphorus pentasulfide. The phosphorus sulfide-hydrocarbon reaction product may be readily obtained by reacting the phosphorus sulfide with the hydrocarbon at a temperature of about 200° F. to about 600° F., and preferably from about 300° F. to about 550° F., using from about 1 to about 10, preferably about 2 to about 5, molecular proportions of hydrocarbon to 1 molecular proportion of the sulfide of phosphorus in the reaction. It is advantageous to maintain a non-oxidizing atmosphere, such as an atmosphere of nitrogen, above the reaction mixture. Usually it is desirable to use an amount of the phosphorus sulfide that will completely react with the hydrocarbon so that no further purification becomes necessary. In the case of monoolefin polymers the preferred ratio is one molecular proportion of the sulfide of phosphorus to two to five molecular proportions of polymer. In such case the reaction is continued until all or substantially all of the phosphorus sulfide has reacted. The reaction time is not critical, and the time required to cause the maximum amount of phosphorus sulfide to react will vary greatly with the temperature. A reaction time of 2 to 10 hours is frequently necessary. If desired, the reaction product may be further treated by blowing with steam, alcohol, ammonia, or an amine at an elevated temperature of about 200° F. to about 600° F. to improve the odor thereof.

The neutralized phosphorus sulfide-hydrocarbon reaction product may then be prepared by reacting the above phosphorus sulfide-hydrocarbon reaction product with the organic basic compound, such as guanidine or guanidine derivative of the type described above. This reaction may be carried out, preferably in a non-oxidizing atmosphere, by contacting the phosphorus sulfide-hydrocarbon reaction product, either as such or dissolved in a suitable solvent such as naphtha, with the basic compound, preferably at a temperature of about 100° F. to 400° F. It is desirable to employ at least enough of the basic compound to neutralize the titratable acidity of the phosphorus sulfide-hydrocarbon product. In practice a somewhat greater amount of basic compound is generally employed, since the basic compound can be reacted in proportions greater than that required for the neutralization of the titratable acidity. When the basic compound is added in the form of a carbonate, the completion of the reaction is indicated by a cessation of carbon dioxide evolution. It has been found that somewhat superior products are formed when a water-soluble basic compound, e. g., guanidine carbonate, is dissolved in or mixed with water when contacted with the phosphorus sulfide-hydrocarbon reaction product. In the case of guanidine carbonate it is preferable to employ a mixture of the salt and water containing 30 to 70% by weight of the salt.

Since the additives of the present invention are to be dissolved in mineral oils, the hydrocarbons which are reacted with a sulfide of phosphorus and the guanyl compounds will be chosen with a view to provide a product which is soluble in the oil base or which has such marginal solubility that it can be plasticized with a high molecular weight alcohol, ester, or other plasticizers.

When additives of the present invention are

## 6

employed in mineral lubricating oils, they are preferably added in proportions of about 0.001 to about 10.0% and preferably 1.0 to about 6.0%. The proportions giving the best results will vary somewhat according to the nature of the additive and the specific purpose which the lubricant is to serve in a given case. For commercial purposes, it is convenient to prepare concentrated oil solutions in which the amount of additive in the composition ranges from 25% to 50% by weight, and to transport and store them in such form. In preparing a lubricating oil composition for use as a crankcase lubricant the additive concentrate is merely blended with the base oil in the required amount.

In certain cases it may be found that the effect of adding compounds of the type described above to a lubricating oil will be to increase the detergent effect of the oil without sufficiently providing oxidation resisting characteristics. In such a case it is advantageous to add to the lubricant, in addition to the additives of the present invention, a substance containing sulfur and/or phosphorus. Elemental sulfur may be used for this purpose or an organic sulfur compound, particularly an organic sulfur compound capable of being decomposed to give free sulfur at a temperature to which the lubricant is subjected during use. Examples of such organic sulfur compounds are sulfurized mineral oils, terpenes, olefins, and diolefins, sulfurized animal and vegetable oils, sulfurized isobutylene polymer, etc.

Below are given detailed descriptions of preparations of examples of lubricating oil additives described above as well as engine tests in which an oil containing the additives was used as the lubricant. It is to be understood that these examples are given as illustrations of the present invention and are not to be construed as limiting the scope thereof in any way.

## Example 1

202 grams (0.8 mol) of octadecene was dissolved in an equal weight of a conventionally refined Coastal distillate oil in a three-necked round bottomed flask equipped with a stirrer, solids addition flask, nitrogen inlet tube, and condenser. The temperature of the mixture was raised to 125° C. and 44 grams (0.2 mol) of phosphorus pentasulfide was added over a period of one hour. The temperature was then raised to 144° C. and maintained at this point for two hours, stirring being continued. The entire reaction was conducted in an atmosphere of nitrogen. The hot solution was filtered to remove a small amount of tarry material.

90 grams of the concentrate of the  $P_2S_5$  treated octadecene prepared as described above was placed in a beaker and heated to 125° C. 11 grams of guanidine carbonate was added over a period of two hours with vigorous stirring. Three drops of silicone fluid was added to minimize foaming during this operation. After the guanidine carbonate was added the temperature was raised to 144° C. and then retained at this point for two hours, after which the solution was filtered.

## Example 2

A guanidine product in the form of a concentrate was prepared in the manner and from the materials described in Example 1, except that in the step of neutralization with guanidine carbonate 88 grams of the concentrate of  $P_2S_5$ -octadecene product was treated with a mixture of 5

grams of guanidine carbonate and 1 gram of water.

*Example 3*

Reactions were carried out as in Example 2, except that a mixture of 5 grams of guanidine carbonate and 7 grams of water was used in the neutralization reaction.

*Example 4*

1200 grams of polyisobutylene of a molecular weight of about 1200 was placed in a three-liter, three-necked round-bottom flask and heated to 300° F. 125 grams of phosphorus pentasulfide was added and the temperature raised to 400° F. over a two-hour period, and heating was continued at this temperature for three more hours with stirring. The mixture was blown with nitrogen for another five hours at 400° F. and then filtered. 200 grams of the phosphorus pentasulfide-treated polyisobutylene thus prepared was dissolved in 200 g. of a solvent extracted Mid-Continent distillate oil of 150 seconds (Saybolt) at 100° F. and treated with 25 g. of guanidine carbonate dissolved in 35 g. of water at 130° C. for three hours and filtered.

*Example 5*

152.5 grams of polyethylene of molecular weight of about 400 was placed in a reaction flask as in Example 4 and heated to 300° F. 30 grams of phosphorus pentasulfide was added and the temperature raised to 400° F. and held at this point for 6½ hours, after which the reaction mixture was filtered. The product was diluted with 150 grams of a solvent extracted Mid-Continent distillate oil of 150 seconds (Saybolt) viscosity at 100° F. 200 grams of this solution was treated at 300° F. with 40 grams of guanidine carbonate dissolved in 100 grams of water and the mixture stirred at this temperature for 3½ hours and filtered.

*Example 6*

150 grams of polybutene-1 having a viscosity of 135 seconds (Saybolt) at 210° F. was placed in a reaction flask and 40 grams of phosphorus pentasulfide added at 300° F. This mixture was then heated at 400° F. for 6½ hours with stirring and filtered. The product was diluted with 150 grams of the solvent oil employed in Example 5. 278 grams of this solution was treated with 20 grams of guanidine carbonate dissolved in 50 grams of water and the mixture heated at 350° F. for 4½ hours and filtered.

*Example 7*

The guanidine products prepared by the methods of Examples 1 to 6 were blended in a lubricating oil base consisting of a solvent extracted Coastal naphthenic oil of 60 seconds viscosity (Saybolt) at 210° F. The blends contained 4 weight % of the concentrates (2 wt. % of active ingredients). The blends were submitted to a standard twenty-hour Lauson engine test, which

was conducted by operating the Lauson engine at 1800 R. P. M. for 20 hours with a 1.5 indicated kilowatt load, 300° F. oil temperature and 295° F. jacket temperature. A similar test was applied to the unblended base oil. The oils were rated by the demerit system, wherein a perfectly clean surface is given a rating of 0, while a rating of 10 is given to the worst condition which could be expected of that surface. The results are shown in the following table:

| Oil Composition                  | Hydrocarbon Reacted with P <sub>2</sub> S <sub>5</sub> | Concentration of Guanidine Carbonate in Aqueous Solution | Piston Skirt Varnish Demerit |
|----------------------------------|--------------------------------------------------------|----------------------------------------------------------|------------------------------|
| Base oil                         | Octadecene                                             | Solid salt                                               | 3.8                          |
| Base oil+2% product of Example 1 | Octadecene                                             | 83%                                                      | 0.8                          |
| Base oil+2% product of Example 2 | Octadecene                                             | 42%                                                      | 0.4                          |
| Base oil+2% product of Example 3 | Polyisobutene                                          | 42%                                                      | 0.0                          |
| Base oil+2% product of Example 4 | Polyisobutene                                          | 39%                                                      | 0.8                          |
| Base oil+2% product of Example 5 | Polyethylene                                           | 39%                                                      | 1.4                          |
| Base oil+2% product of Example 6 | Polybutene-1                                           | 39%                                                      | 1.4                          |

These results show the excellent detergency characteristics of the guanidine products and also show that the use of aqueous solutions of guanidine carbonate gives an improved product over the use of solid guanidine carbonate. The mechanism by which the use of water gives an improved product is not definitely known. However, it is apparently related to the effect of water or steam in causing a decrease in the sulfur content below the theoretical value.

*Example 8*

A blend containing 4% by weight of the 50% concentrate of guanidine product prepared as described in Example 1 (2% of active ingredient) in a solvent extracted paraffinic type of mineral lubricating oil of SAE 30 viscosity grade and a sample of the unblended oil base were employed as the crankcase lubricant in 36 hour tests with a Chevrolet engine operated at 30 brake horsepower, 3150 R. P. M. speed, 280° F. oil temperature and 200° F. jacket temperature. The piston skirt varnish demerit was determined. The results are shown in the following table:

| Lubricant                                           | Varnish Demerit |
|-----------------------------------------------------|-----------------|
| Base Oil                                            | 0.6             |
| Base Oil+2% Active Ingredient, Product of Example 1 | 0.3             |

*Example 9*

A blend containing 4% of the product of Example 1 (2% of active ingredient) in a solvent extracted paraffinic type mineral lubricating oil of SAE 30 viscosity grade and a sample of the unblended base oil were employed as the crankcase lubricant in tests with a Caterpillar diesel engine operated for 120 hours and 6 hours of break-in time for each test, at approximately 19.8 brake horsepower, 1000 R. P. M. speed, 145-150° F. oil-to-bearing temperature, and 175-180° F. water jacket temperature. After each test was completed, the ring zone demerit rating was determined. The results are shown in the following table:

| Lubricant                                           | Ring Zone Demerit |
|-----------------------------------------------------|-------------------|
| Base Oil                                            | 2.1               |
| Base Oil+2% Active Ingredient, Product of Example 1 | 1.1               |

The products of the present invention may be employed not only in ordinary hydrocarbon lubricating oils but also in the "heavy duty" type of lubricating oils which have been compounded with such detergent type additives as metal soaps, metal petroleum sulfonates, metal phenates, metal alcoholates, metal alkyl phenol sulfides, metal organo phosphates, thiophosphates, phosphites and thiophosphites, metal salicylates, metal xanthates and thioxanthates, metal thiocarbamates, amines and amine derivatives, reaction products of metal phenates and sulfur, reaction products of metal phenates and phosphorus sulfides, metal phenol sulfonates and the like. Thus the additives of the present invention may be used in lubricating oils containing such other addition agents as barium tert.-octylphenol sulfide, calcium tert.-amylphenol sulfide, nickel oleate, barium octadecylate, calcium phenyl stearate, zinc diisopropyl salicylate, aluminum naphthenate, calcium cetyl phosphate, barium di-tert.-amylphenol sulfide, calcium petroleum sulfonate, zinc methyl cyclohexyl thiophosphate, calcium dichlorostearate, etc. Other types of additives such as phenols and phenol sulfides may be employed.

The lubricating oil base stocks used in the compositions of this invention may be straight mineral lubricating oils or distillates derived from paraffinic, naphthenic, asphaltic, or mixed base crudes, or, if desired, various blended oils may be employed as well as residuals, particularly those from which asphaltic constituents have been carefully removed. The oils may be refined by conventional methods using acid, alkali and/or clay or other agents such as aluminum chloride, or they may be extracted oils produced, for example, by solvent extraction with solvents of the type of phenol, sulfur dioxide, furfural, dichlorodiethyl ether, nitrobenzene, crotonaldehyde, etc. Hydrogenated oils, white oils, or shale oil may be employed as well as synthetic oils, such as esters and polyethers as well as those prepared, for example, by the polymerization of olefins or by the reaction of oxides of carbon with hydrogen or by the hydrogenation of coal or its products. Also, for special applications, animal, vegetable or fish oils or their hydrogenated or volatilized products may be employed in admixture with mineral oils.

For the best results the base stock chosen should normally be that oil which without the new additive present gives the optimum performance in the service contemplated. However, since one advantage of the additives is that their use also makes feasible the employment of less satisfactory mineral oils or other oils, no strict rule can be laid down for the choice of the base stock. Certain essentials must of course be observed. The oil must possess the viscosity and volatility characteristics known to be required for the service contemplated. The oil must be a satisfactory solvent for the additive, although in some cases auxiliary solvent agents may be used. The lubricating oils, however they may have been produced, may vary considerably in viscosity and other properties depending upon the particular use for which they are desired, but they usually range from about 40 to 150 seconds Saybolt viscosity at 210° F. For the lubricating of certain low and medium speed diesel engines the general practice has often been to use a lubricating oil base stock prepared from naphthenic or aromatic crudes and having a Saybolt viscosity at 210° F. of 45 to 90 seconds and a viscosity index of 0 to 50.

However, in certain types of diesel engine and other gasoline engine service, oils of higher viscosity index are often preferred, for example, up to 75 to 100, or even higher, viscosity index.

In addition to the material to be added according to the present invention, other agents may also be used such as dyes, pour depressors, heat thickened fatty oils, sulfurized fatty oils, organometallic compounds, metallic or other soaps, sludge dispersers, anti-oxidants, thickeners, viscosity index improvers, oiliness agents, resins, rubber, olefin polymers, volatilized fats, volatilized mineral oils, and/or volatilized waxes and colloidal solids such as graphite or zinc oxide, etc. Solvents and assisting agents, such as esters, ketones, alcohols, aldehydes, halogenated or nitrated compounds, and the like may also be employed.

Assisting agents which are particularly desirable as plasticizers and defoamers are the higher alcohols having 8 or more carbon atoms and preferably 12 to 20 carbon atoms. The alcohols may be saturated straight and branched chain aliphatic alcohols such as octyl alcohol ( $C_8H_{17}OH$ ), lauryl alcohol ( $C_{12}H_{25}OH$ ), cetyl alcohol ( $C_{16}H_{33}OH$ ), stearyl alcohol, sometimes referred to as octadecyl alcohol, ( $C_{18}H_{37}OH$ ), heptadecyl alcohol ( $C_{17}H_{35}OH$ ), and the like; the corresponding olefinic alcohols such as oleyl alcohol; cyclic alcohols such as naphthenic alcohols; and aryl substituted alkyl alcohols, for instance, phenyl octyl alcohol, or octadecyl benzyl alcohol; or mixtures of these various alcohols, which may be pure or substantially pure synthetic alcohols. One may also use mixed naturally occurring alcohols such as those found in wool fat (which is known to contain a substantial percentage of alcohols having about 16 to 18 carbon atoms) and in sperm oil (which contains a high percentage of cetyl alcohol); and although it is preferable to isolate the alcohols from those materials, for some purposes wool fat, sperm oil or other natural products rich in alcohols may be used per se. Products prepared synthetically by chemical processes may also be used, such as alcohols prepared by the oxidation of petroleum hydrocarbons, e. g. paraffin wax, petrolatum, etc.

In addition to being employed in lubricants the additives of the present invention may also be used in motor fuels, hydraulic fluids, torque converter fluids, cutting oils, flushing oils, turbine oils or transformer oils, industrial oils, process oils and generally as anti-oxidants in mineral oil products. They may also be used in gear lubricants and greases. Since they are powerful surface active agents, they have practical use in dry cleaning fluids; mineral, spirit and aqueous paints, in flotation agents, and as dispersants for insecticides in aqueous and non-aqueous solutions. They are also valuable anti-oxidants for natural and synthetic rubbers.

What is claimed is:

1. As a new composition of matter a product obtained by reacting one molecular proportion of a phosphorus sulfide with about 1 to about 10 molecular proportions of a hydrocarbon at a temperature of about 200° to about 600° F. and neutralizing the acidic reaction product with an organic basic reacting compound selected from the group consisting of: (1) free bases of the composition



in which R, R' and R'' are each members of the group consisting of hydrogen and hydrocarbon

## 11

radicals containing 1-20 carbon atoms, and (2) basic reacting salts of the aforementioned free bases.

2. A composition according to claim 1 in which R, R' and R'' each represent the same atom or group.

3. A composition according to claim 1 in which R, R' and R'' each represent an alkyl group.

4. A composition according to claim 1 in which R, R' and R'' each represent hydrogen.

5. A composition according to claim 1 in which the phosphorus sulfide-hydrocarbon reaction product is neutralized with guanidine carbonate.

6. A composition according to claim 1 in which the acidic reaction product is obtained by reacting phosphorus pentasulfide with a monoolefin.

7. A composition according to claim 6 in which the monoolefin is polyisobutylene.

8. As a new composition of matter a product obtained by reacting about one molecular proportion of phosphorus pentasulfide with two to five molecular proportions of polyisobutylene at a temperature of about 300 to about 550° F., and then neutralizing the product thus obtained with guanidine carbonate.

9. A composition according to claim 8 in which the guanidine carbonate is added in the form of a mixture with water, such mixture containing 30-70% by weight of guanidine carbonate.

10. The process which comprises reacting one molecular proportion of a phosphorus sulfide with about 1 to about 10 molecular proportions of a hydrocarbon at a temperature of about 200° to about 600° F. and neutralizing the acidic reaction product with an organic basic reacting compound selected from the group consisting of: (1) free bases of the composition



in which R, R' and R'' are each members of the group consisting of hydrogen and hydrocarbon radicals containing 1-20 carbon atoms, and (2) basic reacting salts of the aforementioned free bases.

45

## 12

11. A process according to claim 10 in which the phosphorus sulfide is phosphorus pentasulfide and in which the hydrocarbon is a monoolefin.

12. A process according to claim 11 in which the basic reacting compound is guanidine carbonate.

13. A process according to claim 11 in which the monoolefin is polyisobutylene.

14. A process which comprises reacting about one molecular proportion of phosphorus pentasulfide with two to five molecular proportions of polyisobutylene at a temperature of about 300° to about 550° F., and then neutralizing the product thus obtained with guanidine carbonate.

15. A process according to claim 14 in which the guanidine carbonate is employed in the form of a mixture with water, such mixture containing 30-70% by weight of guanidine carbonate.

16. As a new composition of matter a salt of (1) an acid product obtained by reacting one molecular proportion of a phosphorus sulfide with about one to about ten molecular proportions of a hydrocarbon at a temperature of about 200° to about 600° F. and (2) an organic base of the type



in which R, R' and R'' are each members of the group consisting of hydrogen and hydrocarbon radicals containing 1-20 carbon atoms.

30 MAX W. HILL.

## REFERENCES CITED

The following references are of record in the 35 file of this patent:

## UNITED STATES PATENTS

| Number    | Name             | Date           |
|-----------|------------------|----------------|
| 2,400,786 | Rust             | May 21, 1946   |
| 2,401,733 | Heard            | June 11, 1946  |
| 2,403,474 | Bartleson et al. | July 9, 1946   |
| 2,449,933 | Giammaria        | Sept. 21, 1948 |
| 2,449,934 | Giammaria        | Sept. 21, 1948 |
| 2,506,572 | Bartleson        | May 9, 1950    |

45